

(No Model.)

A. SCHMID.

METHOD OF FORMING LAMINATED CORES FOR ELECTRICAL APPARATUS.

No. 406,858.

Patented July 9, 1889.

Fig. 1.



Fig. 2.



Fig. 4.



Fig. 3.



Witnesses

George Brown Jr.  
James Wm. Smith.

Inventor

ALBERT SCHMID.

By his Attorney, Charles A. Tracy.

# UNITED STATES PATENT OFFICE.

ALBERT SCHMID, OF ALLEGHENY, ASSIGNOR TO THE WESTINGHOUSE ELECTRIC COMPANY, OF PITTSBURG, PENNSYLVANIA.

## METHOD OF FORMING LAMINATED CORES FOR ELECTRICAL APPARATUS.

SPECIFICATION forming part of Letters Patent No. 406,858, dated July 9, 1889.

Application filed May 13, 1889. Serial No. 310,599. (No model.)

*To all whom it may concern:*

Be it known that I, ALBERT SCHMID, a citizen of the Republic of Switzerland, residing in Allegheny, county of Allegheny, and State 5 of Pennsylvania, have invented a certain new and useful Improvement in Method of Forming Laminated Cores for Electrical Apparatus, (Case 319,) of which the following is a specification.

10 My invention relates to certain improvements in the manufacture of cores for electrical apparatus—such, for instance, as the cores of electric inductors or converters, the cores of armatures for electric generators 15 and motors, and other similar apparatus.

It has been found in practice that cores for electrical apparatus which are subjected to a rapid change of magnetic condition are more 20 efficient and less liable to become heated when built of electrically-insulated laminæ of soft iron than when made solid. This is due to the fact that in solid cores the electric currents generated therein circulate within the same. Such currents, while of comparatively 25 low electro-motive force, are of considerable quantity, and are liable to heat the core and render the apparatus less efficient. The use of laminated cores has, therefore, become quite universal. In some instances the 30 adjacent laminæ have been held apart by thin washers, leaving narrow air-spaces between the laminæ. In other instances thin sheets of paper, fiber, or other non-conducting material are placed between the laminæ of soft 35 iron. It is usually desirable that the mass of iron in proximity to the coils of wire applied to a core should be as great as possible. The presence of the insulation between the laminæ lessens somewhat the amount of iron which 40 is contained in a core of given size, and therefore tends to detract from the efficiency of the core. For this reason it is desirable that the insulation between the laminæ should be as thin as possible. The use of washers or 45 thin plates of insulating material is therefore objectionable, because it requires a considerable separation of the successive plates. Another plan is to obtain the insulation by pasting very thin sheets of paper or other insulating material to one surface of the sheets 50 of soft iron from which the laminæ are afterward stamped. In this way very thin insu-

lation may be obtained and the proportion of iron in the core correspondingly increased; but even with this form of insulation the non-conducting material is usually found to occupy about one-sixth as much space as the iron. Another difficulty sometimes encountered in this construction is that the operation of stamping the plates forms a burr along 55 the cut edges, and when the plates are placed together the burrs are liable to pierce through the sheets of paper, and thus destroy to a greater or less extent the insulation between the different plates. The tendency of Foucault or eddy currents to circulate is usually greater near the conducting-wires than in the body of the core, and therefore the presence of the burrs forming electrical connections 60 at the edges is the more objectionable.

The object of the present invention is to overcome these difficulties and to reduce to a minimum the spaces occupied by the insulation, and at the same time to provide a method of manufacturing the core which will secure 75 the required insulation between the laminæ, and shall also cheapen and improve the construction of the core.

The invention consists in first stamping from 80 sheets of suitable magnetizable material—such as soft iron—plates of the required size and form from which to build up the core; then subjecting the plates to an annealing process, which is carried to such an extent that a thin film of oxide is formed over their 85 entire surfaces, and over, also, the burrs or rough edges produced by the stamping process, and afterward building up the core by placing such plates side by side.

The annealing process is carried on in the 90 following manner: The plates are arranged in small piles in a suitable annealing-box. The box is then placed in an oven and gradually heated. This step in practice usually occupies from six to twelve hours. When the 95 proper temperature has been reached, it is kept approximately constant for a sufficient time to produce the required effects. This may vary in different instances; but I usually continue to so heat the plates for about 100 twelve hours. They are then allowed to cool gradually, the heat being gradually lessened. This may occupy a somewhat greater length of time—say from twelve to twenty-four hours.

The gradual cooling secures thoroughly-annealed soft plates. After this treatment the plates are found to be coated with a dark film or very thin scale. This scale consists 5 chiefly of magnetic oxide. It is such a poor conductor of electricity as in effect to amount to an insulator, and at the same time it is more or less magnetic, so that it serves, when the plates are placed together, not only 10 to insulate them from each other, but also as a magnetizable material for the core, thus combining two desirable qualities. At the same time the insulation is extremely thin, and therefore allows the plates themselves to 15 be brought into very close proximity. The thickness of the scale or film is found to be about two ten-thousandths of an inch upon each surface, so that the core consists almost entirely of magnetizable material, and the 20 plates themselves are separated the smallest possible distance. The oxide is very firmly attached to the surfaces of the plates and can only be removed by attrition, so that the plates may be handled without special care 25 and without endangering the insulation.

It is desirable that the plates should be as soft as possible. As already stated, the annealing process has the effect of removing whatever temper may have been given to or 30 remain in the plates, thus softening them and satisfying this requirement. The metal cannot in practice be so perfectly annealed while in the form of large sheets from which the plates are stamped, as it is impossible to heat 35 and cool them evenly; neither can it be thoroughly annealed before it is rolled into sheets, because the subsequent operation of rolling tends to harden it.

In the accompanying drawings, Figure 1 is 40 a side view of a plate employed in building certain forms of converters, such as described, for instance, in Letters Patent No. 366,347, issued July 12, 1887, upon an application filed by me. Fig. 2 is a plan of a converter having 45 a core of the character described. Fig. 3 illustrates an armature-plate, and Fig. 4 an armature-core composed of such plates.

Referring to Figs. 1 and 2, A represents the core of the converter of the construction 50 which it is preferred to employ, and C' C<sup>2</sup> the primary and secondary coils, respectively. The converter may, however, be constructed with a single coil—a portion of the length being designed to be connected in one circuit 55 and a portion in another—or a single coil may be connected entirely in one circuit. The core is composed of thin sheets or plates a', of magnetizable material—such, for instance, as soft iron. In preparing these plates rect- 60 angular plates are stamped with two holes e' e<sup>2</sup>, and these holes are preferably of a rectangular shape and of such size as to receive the coils of wire. Each hole e' e<sup>2</sup> is cut open at f' f<sup>2</sup>. These cuts f' and f<sup>2</sup> may converge, as 65 shown in the figure.

After the plates have been properly stamped their surfaces are oxidized, preferably by be-

ing placed in suitable vessels and gradually heated to a very high temperature. They are kept at such a temperature a proper length of 70 time and then allowed to cool slowly. This step in the process has the double effect of thoroughly annealing and softening the metal and coating the surfaces with a thin film of magnetic oxide. This film also covers the 75 edges and reduces the burrs produced by the stamping, covering them with an insulating material. In this manner the entire surface of each plate is sufficiently insulated to prevent any considerable circulation of Foucault 80 or eddy currents in the core. The plates are then placed one against another, their central tongues being inserted within the coils in the same general manner as described in the patent before referred to, alternate plates 85 being preferably inserted from opposite sides. The manner of building up the core and the shape of the plates may, however, be materially varied without departing from the spirit of my invention.

Figs. 3 and 4 illustrate the construction of the cores of armatures for electric machines. The plates A' are stamped as before, the shape and form being suited to the particular form of armature desired. They are then annealed 95 and thereby softened and coated by a film of insulating oxide, and afterward placed together side by side to form the complete armature-core shown in Fig. 4.

I desire to have it understood that I do not 100 limit my claims to the particular forms of cores here described, nor to the precise periods of heating and cooling, nor the precise methods of oxidizing and annealing set forth in the above specification, and present them 105 as being best suited to illustrate and disclose my invention.

In another application, filed November 6, 1888, Serial No. 290,150, I have described and claimed the cores themselves.

I claim as my invention—

1. The hereinbefore-described method of constructing the cores of electrical apparatus, which consists in first stamping out plates of magnetizable material—such as soft iron— 115 afterward annealing and coating them with an insulating oxide, and building up the core from such annealed plates.

2. The hereinbefore-described method of constructing the laminated cores of electric 120 converters and other electrical apparatus, which consists in first stamping out plates of magnetizable material having the required shape and size, heating such plates after they are so stamped and allowing them to cool 125 gradually, thereby covering their surfaces and edges by coatings of oxide, and afterward building up the core from such plates by placing them face to face, substantially as described.

3. The hereinbefore-described method of constructing the laminated cores of electric converters and other electrical apparatus, which consists in first stamping thin plates

of magnetizable material having the required shape and size, heating such plates after they are so stamped and allowing them to gradually cool, thereby covering their surfaces and edges by coatings of magnetic oxide, and afterward building up the core from such plates by placing them face to face, substantially as described.

4. The hereinbefore-described method of 10 constructing the cores of electrical apparatus, which consists in first stamping out plates of magnetizable material—such as soft iron—afterward coating them with an insulating oxide, and building up the core from such 15 oxidized plates.

5. The hereinbefore-described method of constructing the cores for electrical apparatus, which consists in first stamping out the plates of magnetizable material—such as soft iron—afterward coating the edges of the same 20 with an oxide, and building up the core from such oxidized plates.

In testimony whereof I have hereunto subscribed my name this 7th day of May, A. D. 1889.

ALBERT SCHMID.

Witnesses:

J. M. TATE, Jr.,  
W. D. UPTEGRAFF.